# EUROPEAN PATENT SPECIFICATION

(11) **EP 4 088 611 B1**
(45) Date of publication and mention of the grant of the patent: **17.04.2024**
(21) Application number: 22173089.8
(22) Date of filing: 12.05.2022
(51) Int. Cl.: A43B 13/12, A43B 1/00, A43B 13/36

(54) **METHOD FOR RESOLING A SHOE, AND SHOE**
VERFAHREN ZUR NEUBESOHLUNG EINES SCHUHS UND SCHUH
PROCÉDÉ DE RESSEMELAGE D'UNE CHAUSSURE ET CHAUSSURE

(30) Priority: 13.05.2021 IT 202100012302
(43) Date of publication of application: 16.11.2022
(73) Proprietor: La Sportiva S.P.A., 38030 Ziano di Fiemme (TN) (IT)
(72) Inventor: DELLADIO, Lorenzo, 38030 ZIANO DI FIEMME TN (IT)
(74) Representative: Modiano, Micaela Nadia

(56) References cited:
- FR-A1- 2 957 496
- FR-A1- 3 095 926
- US-A- 3 938 266
- US-A1- 2020 390 188

## Description

The present invention relates to a method for resoling a shoe and to a shoe.

With reference to shoes, such as trekking or climbing boots, it is noted that it is rather usual to consider their resoling during their useful life.

In fact, if one observes that despite the wear of the sole that compromises its use, the upper is still intact and well maintained, one can consider resoling, which can provide for the replacement of the entire sole (therefore both of the tread and of the so-called midsole) or of the tread alone.

In any case, the removal and replacement of the tread alone can be performed effectively only if the shoe has a midsole made of compact material, such as for example a PU (plastic polyurethane) or a so-called "microporous" one, a material of the type of EVA manufactured in sheets and having greater hardness.

Patent FR2957496 describes a method for resoling a shoe, particularly with a sole made of elastomer, which comprises the following successive steps, which consist in: a) heating the sole to a temperature comprised between approximately 40°C and 140°C, depending on the nature of the adhesive material that bonds the superimposed sole layers, so as to soften the bonding agent, b) after the softening of the adhesive material that bonds the sole layers, detaching the lower layer from the upper layer, which corresponds to the worn tread, c) brushing and cleaning with a solvent the lower part of the upper layer of the sole, d) applying a new layer of adhesive material at least on the lower side of the upper layer and/or on the upper face of a new tread, e) reactivating the adhesive material applied in step d) by heating, preferably between 35 and 90°C, depending on the nature of the adhesive material, f) positioning the new tread on the lower side of the upper sole layer, g) pressing together the two sole layers.

If instead the midsole is made of low-density expanded EVA (ethylene vinyl acetate), it is practically impossible to remove the tread (which is bonded with adhesive, during manufacture, to the downward-facing surface of the midsole), since any removal causes the breakage and shattering of the EVA midsole.

While this drawback, in certain types of shoes, such as trekking or climbing boots, is solved by providing for the replacement of the sole in its entirety, i.e., of both the tread and the midsole, in shoes with less structure, such as trekking shoes, approach shoes, hiking shoes or mountain running shoes it is in practice impossible to perform resoling according to the best manufacturing practice.

Moreover, the shoes that more often use expanded EVA as material for providing the midsole are indeed shoes of this type.

Solutions are also known in which the midsole is provided in multiple layers, possibly of different hardness.

In this regard, patent application US2020/390188 describes a shoe in which the midsole is constituted by two platforms: a first platform made of closed-cell foam having different hardness, for example between 50 and 60 Asker C, and a second platform with closed cells having hardness comprised between 35 and 45 Asker C.

Actually, however, these solutions provide for manufacturing the various layers with different hardness in order to obtain synergy during use, furthermore combining hardness with optional recesses in order to obtain a correct shock absorption.

The aim of the present invention is to provide a method for resoling a shoe and a shoe which are capable of improving the background art in one or more of the aspects indicated above.

Within this aim, an object of the invention is to provide a method for resoling a shoe that allows to perform a resoling that it effective and according to best practices also on any shoe with a midsole made of expanded EVA.

Another object of the invention is to provide a shoe that can be resoled easily.

A further object of the invention is to reduce the number of components to be replaced during the resoling process, consequently reducing costs and waste material.

Not least object of the invention is to provide a method for resoling a shoe and a shoe that are highly reliable, relatively easy to provide and at competitive costs.

This aim, these objects and others which will become better apparent hereinafter are achieved by a method for resoling a shoe and by a shoe according to the independent claims, optionally having one or more of the characteristics of the dependent claims.

Further characteristics and advantages will become better apparent from the description of some preferred but not exclusive embodiments of the method for resoling a shoe and of a shoe according to the invention, illustrated by way of non-limiting example in the accompanying drawings, wherein:
Figure 1 is a perspective view of a shoe according to the claimed invention;
Figure 2 is an exploded view of the midsole and the sole;
Figure 3 is an exploded view of the sole used for resoling.

With reference to the figures, the present invention relates first of all to a method for resoling a shoe, generally designated by the reference numeral 10, manufactured by means of a manufacturing method which comprises a step of manufacture of a midsole 2 by co-molding a main body 3 made of expanded EVA which has an Asker C hardness comprised between 40 and 80 on a sheet-like body 4 made of compact EVA which has an Asker A hardness comprised between 70 and 100 and more preferably between 75 and 100.

According to a further aspect, a main body 3 made of expanded EVA has a Shore A hardness comprised between 40 and 80, while the sheet-like body 4 made of compact EVA has a Shore A hardness comprised between 60 and 100.

More generally, the midsole 2 is obtained by co-molding a main body 3 made of expanded material on a sheet-like body 4 made of compact material. More generally, the midsole 2 is obtained by co-molding a main body 3 made of expanded material which has an Asker C hardness comprised between 40 and 80 on a sheet-like body 4 made of compact material which has an Asker A hardness comprised between 70 and 100 and more preferably comprised between 75 and 100.

The step of manufacture of the midsole 2 comprises a step of application, on the face of the sheet-like body 4 made of compact EVA, of a hot-melt bonding agent adapted to facilitate the adhesion of the main body 3 made of expanded EVA.

Preferably, a main body 3 made of expanded EVA has an Asker C hardness comprised between 50 and 60 and the sheet-like body 4 made of EVA which has an Asker A hardness comprised between 80 and 85.

Preferably, a main body 3 made of expanded EVA has a Shore A hardness comprised between 50 and 65, while the sheet-like body 4 made of compact EVA has a Shore A hardness comprised between 70 and 80.

The step of co-molding of the main body 3 on the sheet-like body 4, both made of EVA albeit with different hardness (and therefore densities), allows to obtain a monolithic midsole 2 in which the adhesion between the main body 3 and the sheet-like body 4 is increased further by the chemical compatibility between the materials.

The method then provides for a step of stable mating of the midsole 2, at the face 2b formed by the sheet-like body 4, to a sole 5 and then a step of stable mating of the midsole 2, at its face 2a formed by the main body 3, to an upper 6.

Advantageously, the step of stable mating of the midsole 2 to the sole 5 at the face 2b formed by the sheet-like body 4 comprises an adhesive bonding step.

Preferably, the sheet-like body 4 has a thickness comprised between 0.1 mm and 2 mm and preferably between 0.7 mm and 1.5 mm.

According to an important aspect, the present invention relates to a method for resoling a shoe 10 manufactured by means of the manufacturing method described above.

The resoling method comprises a step of heating the sole 5, so as to bring the sheet-like body 4 to a temperature comprised between 65°C and 85°C, and a step of separation of the sheet-like body 4 from the main body 3.

This heating step for providing the resoling method is performed when the sole 5 is worn or its use is compromised.

A step of stable application of at least one new sole 5a to the main body 3 is then provided.

Preferably, there is a step of stable association of the new sole 5a with a new sheet-like body 4a.

The step of stable application of at least one new sole 5a to the main body 3 comprises an adhesive bonding step.

Advantageously, the step of stable association of the new sole 5a with a new sheet-like body 4a comprises an adhesive bonding step.

According to a further aspect, the present invention relates to a shoe 10 comprising a midsole 2 stably mated on opposite sides to an upper 6 and to a sole 5.

The midsole 2 comprises a main body 3 made of expanded EVA which has an Asker C hardness comprised between 40 and 80 and a sheet-like body 4 made of compact EVA which has an Asker A hardness comprised between 75 and 100.

According to a further aspect, the main body 3 made of expanded EVA has a Shore A hardness comprised between 40 and 80, while the sheet-like body 4 made of compact EVA has a Shore A hardness comprised between 60 and 100.

More generally, the midsole 2 is obtained by co-molding a main body 3 made of expanded material on a sheet-like body 4 made of compact material.

The midsole 2 is mated to the upper 6, at the face 2a formed by the main body 3, and to the sole 5 at the face 2b formed by the sheet-like body 4.

In particular, the main body 3 and the sheet-like body 4 are obtained by co-molding.

In greater detail, the midsole 2 is configured so as to allow the separation of the sheet-like body 4 from the main body 3 following the heating of the sheet-like body 4 to a temperature comprised between 65°C and 85°C.

The present invention provides a shoe which, despite having the midsole made of expanded EVA, can be resoled by removing the sole.

Specifically, by providing the midsole 2 by co-molding a main body 3 made of expanded EVA and a sheet-like body made of compact EVA (which is then stably associated with the sole 5 for example by adhesive bonding) one obtains a solution that allows, if it is necessary to resole the shoe, to remove easily from the main body 3, by heating, the sheet-like body 4 so as to then allow the stable application of a new sole 5a (optionally associated with a new sheet-like element 4a).

It is possible to provide for the possibility to resole the shoe further, by providing for example the possibility to apply stably the new sole 5a (by means of particular adhesives and/or thermal processes) so as to facilitate its subsequent removal.

In practice, the materials used, so long as they are compatible with the specific use, as well as the contingent shapes and dimensions, may be any according to the requirements and the state of the art.

## Claims

1. A method for resoling shoes (10) manufactured by means of a method comprising a step for the manufacture of a midsole (2) by co-molding a main body (3) made of expanded EVA which has an Asker C hardness comprised between 40 and 80 or a Shore A hardness comprised between 40 and 80 on a sheet-like body (4) made of compact EVA which has an Asker A hardness comprised between 70 and 100 or a Shore A hardness comprised between 60 and 100, a step of stable mating of said midsole (2) to a sole (5) at the face (2b) formed by said sheet-like body (4), and to an upper (6) at the face (2a) formed by said main body (3), a step of resoling said shoe (10) manufactured according to said method for the manufacture of shoes (10) being provided which comprises a step of heating said sole (5) until said sheet-like body reaches a temperature comprised between 65°C and 85°C, a step of separating said sheet-like body (4) from said main body (3), and a step of stable application of at least one new sole (5a) to said main body (3).

2. The method according to claim 1, **characterized in that** said sheet-like body (4) made of compact EVA has an Asker A hardness comprised between 70 and 100.

3. The method according to one or more of the preceding claims, **characterized in that** said step of stable mating of said midsole (2) to said sole (5) at said face (2b) formed by said sheet-like body (4) comprises an adhesive bonding step.

4. The method according to one or more of the preceding claims, **characterized in that** said sheet-like body (4) has a thickness comprised between 0.1 mm and 2 mm.

5. The method according to one or more of the preceding claims, **characterized in that** it comprises a step of stable association of said new sole (5a) with a new sheet-like body (4a).

6. The method according to one or more of the preceding claims, **characterized in that** said step of stable application of said at least one new sole (5a) to said main body (3) comprises an adhesive bonding step.

7. The method according to one or more of the preceding claims claim 5, **characterized in that** said step of stable association of said new sole (5a) with said new sheet-like body (4a) comprises an adhesive bonding step.

8. A shoe (10) comprising a midsole (2) stably mated on opposite sides to an upper (6) and a sole (5), **characterized in that** said midsole comprises a main body (3) made of expanded EVA which has an Asker C hardness comprised between 40 and 80 or a Shore A hardness comprised between 40 and 80 and a sheet-like body (4) made of compact EVA which has an Asker A hardness comprised between 70 and 100 or a Shore A hardness comprised between 60 and 100, said midsole (2) being mated to said upper (6), at the face (2a) formed by said main body (3), and to said sole (5) at the face (2b) formed by said sheet-like body (4), said midsole (2) being configured so as to allow the separation of said sheet-like body (4) from said main body (3) as a consequence of the heating of said sheet-like body (4) to a temperature comprised between 65°C and 85°C.

9. The shoe (10) according to claim 8, **characterized in that** said main body (3) and said sheet-like body (4) are obtained by co-molding.

10. The shoe (10) according to claim 8, **characterized in that** said sheet-like body (4) made of EVA has an Asker A hardness comprised between 75 and 100.

## Patentansprüche

1. Ein Verfahren zur Neubesohlung von Schuhen (10), die mit Hilfe eines Verfahrens hergestellt werden, das Folgendes umfasst: einen Schritt des Herstellens einer Zwischensohle (2) durch Überformen eines Hauptkörpers (3) aus geschäumtem EVA, der eine Asker C-Härte zwischen 40 und 80 oder eine Shore A-Härte zwischen 40 und 80 hat, auf einen lagenartigen Körper (4) aus kompaktem EVA, der eine Asker A-Härte zwischen 70 und 100 oder eine Shore A-Härte zwischen 60 und 100 hat; einen Schritt des festen Koppelns der Zwischensohle (2) mit einer Sohle (5) an der Fläche (2b), die durch den lagenartigen Körper (4) gebildet wird, und mit einem Schaft (6) an der Fläche (2a), die durch den Hauptkörper (3) gebildet wird; wobei ein Schritt des Neubesohlens des Schuhs (10) bereitgestellt wird, der nach dem Verfahren zur Herstellung von Schuhen (10) hergestellt wird; welcher Folgendes umfasst: einen Schritt des Erhitzens der Sohle (5), bis der lagenartige Körper eine Temperatur erreicht, die zwischen 65°C und 85°C beträgt; einen Schritt des Trennens des lagenartigen Körpers (4) von dem Hauptkörper (3) und einen Schritt des festen Aufbringens mindestens einer neuen Sohle (5a) auf den Hauptkörper (3).

2. Das Verfahren gemäß Anspruch 1, **dadurch gekennzeichnet, dass** der lagenartige Körper (4) aus kompaktem EVA eine Asker A-Härte zwischen 70 und 100 hat.

3. Das Verfahren gemäß einem oder mehreren der obigen Ansprüche, **dadurch gekennzeichnet, dass** der Schritt des festen Koppelns der Zwischensohle (2) mit der Sohle (5) an der Fläche (2b), die durch den lagenartigen Körper (4) gebildet wird, einen Klebeschritt umfasst.

4. Das Verfahren gemäß einem oder mehreren der obigen Ansprüche, **dadurch gekennzeichnet, dass** der lagenartige Körper (4) eine Dicke zwischen 0,1 mm und 2 mm hat.

5. Das Verfahren gemäß einem oder mehreren der obigen Ansprüche, **dadurch gekennzeichnet, dass** es einen Schritt des festen Verbindens der neuen Sohle (5a) mit einem neuen lagenartigen Körper (4a) umfasst.

6. Das Verfahren gemäß einem oder mehreren der obigen Ansprüche, **dadurch gekennzeichnet, dass** der Schritt des festen Aufbringens der mindestens einen neuen Sohle (5a) auf den Hauptkörper (3) einen Klebeschritt umfasst.

7. Das Verfahren gemäß einem oder mehreren der obigen Ansprüche Anspruch 5, **dadurch gekennzeichnet, dass** der Schritt des festen Verbindens der neuen Sohle (5a) mit dem neuen lagenartigen Körper (4a) einen Klebeschritt umfasst.

8. Ein Schuh (10), der eine Zwischensohle (2) umfasst, welche an gegenüberliegenden Seiten fest mit einem Schaft (6) und mit einer Sohle (5) gekoppelt ist; **dadurch gekennzeichnet, dass** die Zwischensohle einen Hauptkörper (3) aus geschäumtem EVA umfasst, der eine Asker C-Härte zwischen 40 und 80 oder eine Shore A-Härte zwischen 40 und 80 hat, und einen lagenartigen Körper (4) aus kompaktem EVA, der eine Asker A-Härte zwischen 70 und 100 oder eine Shore A-Härte zwischen 60 und 100 hat; wobei die Zwischensohle (2) an der Fläche (2a), die durch den Hauptkörper (3) gebildet ist, mit dem Schaft (6) und an der Fläche (2b), die durch den lagenartigen Körper (4) gebildet ist, mit der Sohle (5) gekoppelt ist; wobei die Zwischensohle (2) ausgebildet ist, um die Trennung des lagenartigen Körpers (4) von dem Hauptkörper (3) infolge der Erhitzung des lagenartigen Körpers (4) auf eine Temperatur zwischen 65°C und 85°C zu gestatten.

9. Der Schuh (10) gemäß Anspruch 8, **dadurch gekennzeichnet, dass** der Hauptkörper (3) und der lagenartige Körper (4) durch Überformen hergestellt werden.

10. Der Schuh (10) gemäß Anspruch 8, **dadurch gekennzeichnet, dass** der lagenartige Körper (4) aus EVA eine Asker A-Härte zwischen 75 und 100 hat.

## Revendications

1. Procédé pour ressemeler des chaussures (10) fabriquées au moyen d'un procédé comprenant une étape pour la fabrication d'une semelle intermédiaire (2) par co-moulage d'un corps principal (3) réalisé avec de l'EVA expansé qui a une dureté Asker C comprise entre 40 et 80 ou une dureté Shore A comprise entre 40 et 80 sur un corps en forme de feuille (4) réalisé à partir d'EVA compact qui a une dureté Asker A comprise entre 70 et 100 ou une dureté Shore A comprise entre 60 et 100, une étape de couplage stable de ladite semelle intermédiaire (2) à une semelle (5) au niveau de la face (2b) formée par ledit corps en forme de feuille (4) et à une tige (6) au niveau de la face (2a) formée par ledit corps principal (3), une étape de ressemelage de ladite chaussure (10) fabriquée selon ledit procédé pour la fabrication de chaussures (10) étant prévue qui comprend une étape pour chauffer ladite semelle (5) jusqu'à ce que ledit corps en forme de feuille atteigne une température comprise entre 65°C et 85°C, une étape pour séparer ledit corps en forme de feuille (4) dudit corps principal (3), et une étape d'application stable d'au moins une nouvelle semelle (5a) sur ledit corps principal (3).

2. Procédé selon la revendication 1, **caractérisé en ce que** ledit corps en forme de feuille (4) réalisé à partir d'EVA compact a une dureté Asker A comprise entre 70 et 100.

3. Procédé selon une ou plusieurs des revendications précédentes, **caractérisé en ce que** ladite étape de couplage stable de ladite semelle intermédiaire (2) à ladite semelle (5) au niveau de ladite face (2b) formée par ledit corps en forme de feuille (4) comprend une étape de liaison adhésive.

4. Procédé selon une ou plusieurs des revendications précédentes, **caractérisé en ce que** ledit corps en forme de feuille (4) a une épaisseur comprise entre 0,1 mm et 2 mm.

5. Procédé selon une ou plusieurs des revendications précédentes, **caractérisé en ce qu'**il comprend une étape d'association stable de ladite nouvelle semelle (5a) avec un nouveau corps en forme de feuille (4a).

6. Procédé selon une ou plusieurs des revendications précédentes, **caractérisé en ce que** ladite étape d'application stable de ladite au moins une nouvelle semelle (5a) sur ledit corps principal (3) comprend une étape de liaison adhésive.

7. Procédé selon une ou plusieurs des revendications précédentes, selon la revendication 5, **caractérisé en ce que** ladite étape d'association stable de ladite nouvelle semelle (5a) avec ledit nouveau corps en forme de feuille (4a) comprend une étape de liaison adhésive.

8. Chaussure (10) comprenant une semelle intermédiaire (2) couplée, de manière stable, sur les côtés opposés, à une tige (6) et à une semelle (5), **caractérisée en ce que** ladite semelle intermédiaire comprend un corps principal (3) réalisé à partir d'EVA expansé qui a une dureté Asker C comprise entre 40 et 80 ou une dureté Shore A comprise entre 40 et 80 et un corps en forme de feuille (4) réalisé à partir d'EVA compact qui a une dureté Asker A comprise entre 70 et 100 ou une dureté Shore A comprise entre 60 et 100, ladite semelle intermédiaire (2) étant couplée à ladite tige (6), au niveau de la face (2a) formée par ledit corps principal (3), et à ladite semelle (5) au niveau de la face (2b) formée par ledit corps en forme de feuille (4), ladite semelle intermédiaire (2) étant configurée afin de permettre la séparation dudit corps en forme de feuille (4) dudit corps principal (3) en conséquence du chauffage dudit corps en forme de feuille (4) à une température comprise entre 65°C et 85°C.

9. Chaussure (10) selon la revendication 8, **caractérisée en ce que** ledit corps principal (3) et ledit corps en forme de feuille (4) sont obtenus par co-moulage.

10. Chaussure (10) selon la revendication 8, **caractérisée en ce que** ledit corps en forme de feuille (4) réalisé à partir d'EVA a une dureté Asker A comprise entre 75 et 100.
